

# United States Patent [19]

Riester et al.

[11] 3,816,141

[45] June 11, 1974

[54] FOGGED, DIRECT POSITIVE SILVER HALIDE EMULSION SENSITIZED WITH AN ISOINDOLINONE POLYMETHINE DYE

[75] Inventors: Oskar Riester, Leverkusen; Hans Öhlschläger, Bergisch-Gladbach, Schildgen, both of Germany

[73] Assignee: Agfa-Gevaert Aktiengesellschaft, Leverkusen, Germany

[22] Filed: July 12, 1972

[21] Appl. No.: 271,152

[30] Foreign Application Priority Data

July 14, 1971 Germany 2135153

[52] U.S. Cl. 96/137, 96/107, 96/108

[51] Int. Cl. G03c 1/08, G03c 1/28

[58] Field of Search 96/137, 140, 107, 108

[56] References Cited  
UNITED STATES PATENTS

3,687,674 8/1972 Sato et al. 96/101  
3,687,675 8/1972 Gaugh 96/107

Primary Examiner—Ronald H. Smith

Assistant Examiner—Won H. Louie, Jr.

Attorney, Agent, or Firm—Connolly and Hutz

[57] ABSTRACT

Light-sensitive photographic direct positive material containing at least one fogged silver halide emulsion layer which layer contains a polymethine sensitizer containing an isoindolinone ring.

1 Claim, 5 Drawing Figures



PATENTED JUN 11 1974

3,816,141

FIG. 1



FIG. 2



FIG. 3



FIG. 4



FIG. 5



**FOGGED, DIRECT POSITIVE SILVER HALIDE  
EMULSION SENSITIZED WITH AN  
ISOINDOLINONE POLYMETHINE DYE**

This invention is related to photographic direct positive silver halide emulsions which are spectrally sensitized with polymethine sensitizers which contain an isoindolinone ring. 5

Numerous sensitizing dyes are known for sensitizing the usual negative silver halide emulsions, e.g., mono- or trimethine cyanines, merocyanines or rhodacyanines. 10

The known sensitizing dyes, however, cannot usually be used for sensitizing direct positive emulsions, i.e., emulsions which are processed to produce positive images after the usual exposure and development, because they generally cause flattening of the gradation. 15 On the other hand, compounds have already been described which can only be used as sensitizing dyes for direct positive emulsions. In negative emulsions, these compounds cause fogging and their sensitizing effect is unsatisfactory. Indocyanines, for example, have been used as sensitizing dyes for direct positive emulsions. 20 They are quite suitable sensitizers for the red region of the spectrum but their sensitizing effect is still not quite sufficient. The same applies to the direct positive indole sensitizing dyes for the green region of the spectrum and to the bis-thiazolyl and bis-selenazolyl compounds which are known as direct positive sensitizing dyes. 25

It is among the objects of the present invention to provide sensitizing dyes for direct positive silver halide emulsions which have a sufficiently intense sensitizing effect and have no disadvantageous effect on the gradation. 30

We now have found a photographic material containing at least one direct positive silver halide emulsion layer which is spectrally sensitized with polymethine sensitizers containing an isoindolinone ring. 35

Sensitizers of the following formula are particularly suitable: 40



wherein

R<sup>1</sup> represents (1) a saturated or unsaturated aliphatic group which preferably contains up to six carbon atoms and which may be substituted, e.g., with phenyl, hydroxyl or halogen such as chlorine or bromine, or (2) aryl, preferably phenyl, which also may be substituted, e.g., with an alkyl or alkoxy group which preferably has up to three carbon atoms or with halogen such as fluorine, chlorine or bromine; 55

R<sup>2</sup> is hydrogen or halogen such as chlorine, bromine or iodine; 60

R<sup>3</sup> represents (1) a saturated or unsaturated aliphatic group which preferably contains up to 6 carbon atoms which may be substituted, e.g. with phenyl, hydroxyl or halogen such as fluorine, chlorine or bromine, carboxyl, esterified carboxyl, carbamoyl, sulfo or an esterified sulfo group, (2) cycloalkyl such as cyclohexyl or (3) aryl, in particular phenyl which also may be substituted, e.g. with alkyl or alkoxy having preferably up to three carbon atoms or halogen such as chlorine, bromine or iodine; 65

n is 0 or 1;

X<sup>⊖</sup> stands for anion, e.g. a halide such as chloride, bromide or iodide, perchlorate, sulfate, methylsulfate, p-toluenesulfonate;

Q represents the ring members required for completing a 5- or 6-membered heterocyclic ring; the heterocyclic group may contain a condensed benzene or naphthalene ring and additional substituents; the heterocyclic groups may be those commonly found in cyanine chemistry, for example those based on thiazole (e.g., thiazole, 4-methylthiazole, 5-methylthiazole, 4,5-dimethylthiazole, 4-phenylthiazole, 5-phenylthiazole or 4,5-diphenylthiazole), benzothiazole (e.g., benzothiazole, 4-chlorobenzothiazole, 5-chlorobenzothiazole, 6-chlorobenzothiazole, 7-chlorobenzothiazole, 6-bromobenzothiazole, 5-iodobenzothiazole, 6-iodobenzothiazole, 4-methylbenzothiazole, 5-methylbenzothiazole, 6-methylbenzothiazole, 5,6-dimethylbenzothiazole, 4-phenylbenzothiazole, 5-phenylbenzothiazole, 6-phenylbenzothiazole, 5-hydroxybenzothiazole, 6-hydroxybenzothiazole, 4-methoxybenzothiazole, 5-methoxybenzothiazole, 6-methoxybenzothiazole, 5-ethoxybenzothiazole, 6-ethoxybenzothiazole, 5,6-dimethoxybenzothiazole, 5,6-methylenedihydroxy-benzothiazole, 5-diethylaminobenzothiazole, 6-diethylaminobenzothiazole, 6-nitro-benzothiazole, 5-carboxybenzothiazole, 5-sulfonybenzothiazole, 6-cyanobenzothiazole, 5-trifluoromethylbenzothiazole, 5-benzoylbenzothiazole, tetrahydrobenzothiazole or 7-oxo-tetrahydrobenzothiazole), naphthothiazole (e.g. naphtho[1,2-d]thiazole, naphtho[2,1-d]thiazole, 7-methoxy-naphtho[2,1-d]thiazole or 8-methoxynaphtho[1,2-d]thiazole), selenazole (e.g. 4-methylselenazole or 4-phenylselenazole), benzoselenazole (e.g., benzoselenazole, 5-chlorobenzoselenazole, 5,6-dimethylbenzoselenazole, 5-hydroxy-benzoselenazole, 5-methoxy-benzoselenazole or tetrahydrobenzoselenazole), naphthoselenazole (e.g. naphtho[1,2-d]selenazole or naphtho[2,1-d]selenazole), oxazole (e.g. oxazole, 4-methyloxazole, 4-phenyloxazole or 4,5-diphenyloxazole), benzoxazole (e.g., benzoxazole, 5-chlorobenzoxazole, 6-chlorobenzoxazole, 5,6-dimethylbenzoxazole, 5-phenylbenzoxazole, 5-hydroxybenzoxazole, 5-methoxybenzoxazole, 5-ethoxybenzoxazole, 6-dialkylaminobenzoxazole, 5-carboxybenzoxazole, 5-sulfonybenzoxazole, sulfonamidobenzoxazole or 5-carboxyvinylbenzoxazole), naphthoxazole (e.g., naphtho[1,2-d]oxazole, naphtho[2,1-d]oxazole or naphtho[2,3-d]oxazole), 3,3-dialkylindolenine (e.g., 3,3-dimethylindolenine, 3,3,5-trimethylindolenine or 3,3-dimethyl-5-methoxyindolenine), 2-pyridine (e.g., pyridine, 3-methylpyridine, 4-

3

methylpyridine, 5-methylpyridine, 6-  
 methylpyridine, 3,4-dimethylpyridine, 3,5-  
 dimethylpyridine, 3,6-dimethylpyridine, 4,5-  
 dimethylpyridine, 4,6-dimethylpyridine, 4-  
 chloropyridine, 5-chloropyridine, 6- 5  
 chloropyridine, 3-hydroxypyridine, 4-  
 hydroxypyridine, 5-hydroxypyridine, 3-  
 phenylpyridine, 4-phenylpyridine or 6-  
 phenylpyridine), 4-pyridine (e.g. 2-methylpyridine,  
 3-methylpyridine, 2,3-dimethylpyridine, 2,5- 10  
 dimethylpyridine, 2,6-dimethylpyridine, 2-  
 chloropyridine, 3-chloropyridine, 2-  
 hydroxypyridine or 3-hydroxypyridine), 2-  
 quinoline (e.g., quinoline, 3-methylquinoline, 5-  
 methylquinoline, 7-methylquinoline, 8- 15  
 methylquinoline, 6-chloroquinoline, 8-  
 chloroquinoline, 6-methoxyquinoline, 6-  
 ethoxyquinoline, 6-hydroxyquinoline, 8-  
 hydroxyquinoline or 5-oxo-5,6,7,8-  
 tetrahydroquinoline), 4-quinoline (e.g., quinoline, 20

4

6-methoxyquinoline, 7-methylquinoline or 8-  
 methylquinoline), isoquinoline (e.g., isoquinoline  
 or 3,4-dihydroisoquinoline), thiazoline (e.g., thiaz-  
 oline or 4-methylthiazole), oxazolone and hetero-  
 cyclic groups of the pyrrole, tetrahydropyridine,  
 thiadiazole, oxadiazole, pyrimidine, triazine or  
 benzothiazine and pyrimidone or thiopyrimidone.  
 The aryl groups and heterocyclic groups may carry  
 any other additional substituents, e.g., alkyl groups  
 which preferably contain up to three carbon atoms  
 such as methyl or ethyl, halogen such as chlorine  
 or bromine, hydroxyl, alkoxy preferably with up to  
 three carbon atoms such as methoxy or ethoxy, hy-  
 droxyalkyl, alkylthio, aryl such as phenyl, aralkyl  
 such as benzyl, amino, substituted amino or nitro.

The following are examples of suitable compounds.  
 The absorption maxima are measured in methanolic  
 solution unless otherwise indicated. In the table,  
 ACOH means glacial acetic acid and DMSO dimethyl-  
 sulfoxid.

## Compound

Absorption Sensitization  
 maximum maximum  
 (nm) (nm)

1



458 555



2



490 585

3



481 575

Compound

Absorption  
maximum  
(nm)

Sensiti-  
zation  
maximum  
(nm)

| 4 |    | 472<br>(ACOH)    | 565 |  |
|---|-------------------------------------------------------------------------------------|------------------|-----|--|
| 5 |   | 431<br>$J^-$     | 510 |  |
| 6 |  | 449<br>$J^-$     | 545 |  |
| 7 |  | 450<br>$ClO_4^-$ | 545 |  |

## Compound

Absorption  
maximum  
(nm)

Sensiti-  
zation  
maximum  
(nm)



| Compound |                                                                                     | Absorption<br>maximum<br>(nm) | Sensitization<br>maximum<br>(nm) |
|----------|-------------------------------------------------------------------------------------|-------------------------------|----------------------------------|
| 13       |    | 490                           | 580                              |
| 14       |   | 474                           | 570                              |
| 15       |  | 468                           | 550                              |
| 16       |  | 460                           | 550                              |

| Compound |                                                                                     | Absorption<br>maximum<br>(nm) | Sensitization<br>maximum<br>(nm) |
|----------|-------------------------------------------------------------------------------------|-------------------------------|----------------------------------|
| 17       |    | 454                           | 550                              |
| 18       |   | 462                           | 560                              |
| 19       |  | 463<br>(DMSO)                 | 540                              |
| 20       |  | 480<br>(Aceton)               | 550                              |

## Compound

Absorption  
maximum  
(nm)      Sensitization  
maximum  
(nm)

|    |  |                 |     |
|----|--|-----------------|-----|
| 21 |  | 481<br>(ACOH)   | 570 |
| 22 |  | 464<br>(DMSO)   | 545 |
| 23 |  | 470             | 560 |
| 24 |  | 470<br>(Aceton) | 565 |

## Compound

Absorption  
maximum  
(nm)Sensitization  
maximum  
(nm)

425

495

 $\text{ClO}_4^-$ 

419

490

 $\text{J}^-$ 

437

520

 $\text{J}^-$ 

434

520

 $\text{H}_3\text{C}-\text{C}_6\text{H}_4-\text{SO}_3^-$

| Compound | Absorption<br>maximum<br>(nm) | Sensitization<br>maximum<br>(nm) |
|----------|-------------------------------|----------------------------------|
|----------|-------------------------------|----------------------------------|



(Aceton)



(Aceton)



## Compound

| Absorption maximum (nm) | Sensitization maximum (nm) |
|-------------------------|----------------------------|
|-------------------------|----------------------------|



486

580

The dyes are prepared by condensation of N-substituted 3-formylmethyleneisoindolinones with 2-methyl-quaternary salts of heterocyclic nitrogen bases as described by H. R. MÜLLER and M. SEE-FELDER in "Liebigs Ann. Chem." 728, 88 - 98 (1969).

The dyes to be used according to the invention generally have no sensitizing effect in ordinary negative emulsions but on the contrary reduce the total sensitivity and reinforce the unwanted grey fog. In direct positive emulsions, on the other hand, these dyes have a spectral sensitizing effect resulting in exceptionally high sensitivity and excellent steepness of the gradation.

Silver halide emulsions sensitized with the present dyes are not or only slightly colored so that they can also be used coated on paper supports. The emulsions may be fogged by the usual methods, for example by the action of light or so-called chemical fogging agents, for example stannous chloride, formaldehyde, thiourea dioxide. Another advantageous method of fogging the emulsions consists in adding a reducing compound, for example thiourea dioxide, and the compound of a metal which is more electropositive than silver, for example a gold salt, e.g. potassium chloroaurate, as described in British Pat. Specification No. 723,019.

Typical reducing compounds which are suitable for preparing such fogged silver halide emulsions are, for example, stannous salts, such as stannous chloride, hydrazine, sulfur compounds such as thiourea dioxide, phosphonium salts, e.g., tetra(hydroxymethyl)-phosphonium chloride. Typical compounds of metals which are more electropositive than silver are, for example, compounds of gold, rhodium, platinum, palladium and iridium. It is preferred to use soluble salts of the said noble metals, e.g., potassium chloroaurate, auric chloride and  $(\text{NH}_4)_2\text{PdCl}_6$ .

The concentration of the reducing agents or the compounds of the metal which is more electropositive than silver used for fogging can vary within wide limits. In general, concentrations of 0.0005 to about 0.06 milliequivalents of reducing agent and about 0.001 to about 0.01 milli-mols of the noble metal salt per mol silver halide have proved sufficient.

Fogging can be also accomplished with the method of silver halide digestion described by WOOD in

"J.phot.Science" 1 (1963) page 163, at pAg values between 2 and 5 and pH values of about 6.5.

Any type of direct positive photographic emulsions can be spectrally sensitized by the sensitizing dyes of the present invention. Suitable direct positive emulsions include silver halide emulsions the grains of which have high internal sensitivity in particular silver halide emulsions containing internal electron traps. Particular utility is exhibited by direct positive silver halide grains comprising a central core of a silver halide which contains centres which act as electron traps and an outer shell covering said core comprising a fogged silver halide that develops to silver without exposure. Emulsions of that type are disclosed by E. MOISAR and F. WAGNER in "Berichte der Bunsengesellschaft fur physikalische Chemie" 67 (1963), pages 356 - 359. We furthermore refer to British Pat. specifications Nos. 1,027,146 and 1,151,781 or to French Pat. specification No. 1,585,791. The formations of the centres or specks in the inside of the grains particularly on the core of the composite grain are produced as known per se by chemical sensitizing the emulsion with compounds of noble metals in particular gold or iridium salts are sulfur compounds such as thiosulfates. In particular useful is a treatment with noble metal salts and sulfur compounds.

The spectral sensitizers of the present invention can also be applied to direct positive emulsions which are fogged on the surface so that they can be developed to silver without exposure and which contain at the surface electron acceptors such as desensitizing dyes. Suitable dyes for this purpose are wellknown. Reference is made, e.g., to pinacrytol yellow or nitrosubstituted polymethine dyes. The technic of desensitization and the chemical structure of suitable desensitizing dyes are described e.g., by O. RIESTER in "Mitteilungen aus den Forschungslaboratorien der Agfa," Volume 1 (1955), page 44 or in the handbook "Grundlagen der photographischen Prozesse mit Silberhalogeniden", Volume 3, page 1077. The direct positive sensitizing dyes of the present invention can be used in combination with further sensitizing dyes capable of sensitizing direct positive emulsions and desensitizing negative silver halide emulsions as described, for example, in U.S. Pat. specifications Nos. 3,314,796 or 3,505,070.

Further suitable direct positive emulsion are described in German Pat. specifications Nos. 606,392 or

642,222 or in UK Pat. specifications Nos. 581,773 or 655,009.

The direct positive emulsions may also contain mercury salts and thallium salts as described in British Pat. specification No. 1,203,744 or U.S. Pat. specification No. 3,620,750.

The silver halide of the silver halide emulsions to which the new cyanine dyes may be added may consist of one of the usual silver halides used for preparing photographic silver halide emulsions, i.e., for example silver bromide, silver iodide, silver chloride, silver chlorobromide, silver bromoiodide and silver chlorobromiodide.

The new dyes may be incorporated with silver halide emulsions at the usual concentrations, for example concentrations of about 50 to 2,000 mg, preferably about 400 to 800 mg/mol of silver halide.

The new cyanine dyes are preferably added to the washed silver halide emulsions and dispersed in them as uniformly as possible. The incorporation of the dyes in the emulsions may be carried out by the usual known methods, for example, the dyes may be added to the emulsions from solutions in suitable solvents. The solvents must, of course, be selected so that they have no adverse effect on the light-sensitive photographic material which is to be produced. Suitable solvents are, for example, methanol, isopropanol, acetone and water, either separately or mixed with each other.

The binder of the silver halide emulsions to which the cyanine dyes according to the invention may be added may be any of the hydrophilic colloids commonly used for the preparation of photographic silver halide emulsions, for example, natural substances such as proteins, in particular gelatin, albumin, agar-agar, gum arabic or alginic acid or synthetic hydrophilic resins such as polyvinyl alcohol, polyvinyl pyrrolidone, cellulose ethers or partly hydrolyzed cellulose acetate.

The emulsions containing one or more cyanine dyes according to the invention may be applied to the usual opaque or transparent photographic supports used for the preparation of photographic materials, for example supports of glass, cellulose acetate, cellulose acetobutyrate or polyesters, e.g., polyethylene terephthalate, or supports of baryta-coated paper or paper coated with polyolefines such as polyethylene.

The photographic silver halide emulsions to which the new cyanine dyes are added, as well as the other layers of a photographic material which is prepared using these emulsions may be hardened by the addition of the usual hardeners such as aldehyde hardeners, e.g., formaldehyde or mucochloric acid.

The good sensitizing effect is preserved even in the presence of water-soluble and emulsified color couplers. The emulsion may also contain the usual wetting agents, stabilizers, brightening agents and other additives.

#### EXAMPLE

45 mg of sensitizer 3 in the form of a 1:1000 solution in methanol are added with stirring to 1 kg of a direct positive emulsion which has been prepared by chemical fogging using ammonia and excess silver nitrate and which contains 0.4 mol of silver bromide per kg of casting solution with an iodine content of 2.5 mol percent, based on the amount of silver, and the mixture is left to digest for 10 minutes. 10 ml of a 4 percent aqueous solution of saponin as wetting agent and 25 ml of a 5

percent solution of mucochloric acid are then added. The emulsion is then cast on a support of cellulose acetate in the usual manner.

When dry, the layer is exposed to white light through a test wedge in a sensitometer customarily employed in the art and developed for 5 minutes at 20°C using a developer of the following composition:

|    |                                |        |
|----|--------------------------------|--------|
| 10 | p-methylaminophenol            | 3.5 g  |
|    | anhydrous sodium sulfite       | 60.0 g |
|    | hydroquinone                   | 9.0 g  |
|    | anhydrous sodium carbonate     | 40.0 g |
|    | potassium bromide              | 3.5 g  |
|    | made up to 1 litre with water. |        |

15 The layer is then fixed with an aqueous solution of sodium thiosulfate in the usual manner.

20 A positive image of the test wedge with exceptional whites and an excellent gamma value (gradation) is obtained. The spectral sensitization curve is represented in FIG. 2.

25 FIG. 1 shows for comparison the sensitivity curve obtained without sensitizer.

When sensitizer 3 is replaced by an equal quantity of compound 8, the sensitization curve of FIG. 3 is obtained, and when an equal quantity of compound 9 is used, the sensitization curve of FIG. 4 is obtained. The sensitization curve of FIG. 5 is obtained when using compound 17 in the same way.

We claim:

1. Light-sensitive photographic direct positive material containing at least one fogged silver halide emulsion layer which layer contains an isoindolinone polymethine sensitizer of the following formula:



45

in which

R<sup>1</sup> represents an aliphatic group having up to 6 carbon atoms or a phenyl group;

R<sup>2</sup> stands for hydrogen or halogen;

R<sup>3</sup> represents an aliphatic group having up to 6 carbon atoms, cycloalkyl or aryl;

n is 0 or 1;

X<sup>-</sup> represents any anion;

Q stands for the ring members required for completing a 5- or 6-membered heterocyclic ring based on thiazole, benzothiazole, naphthothiazole, selenazole, benzoselenazole, naphthoselenazole, oxazole, benzoxazole, naphthoxazole, 3,3-dialkylindoline, 2-pyridine, 4-pyridine, 2-quinoline, 4-quinoline, isoquinoline, thiazoline, oxazoline, pyrrolidine, tetrahydropyridine, thiadiazole, oxadiazole, pyrimidine, triazine, benzothiazine, pyrimidone or thiopyrimidone, which heterocyclic ring may contain a fused benzene or naphthalene ring.

\* \* \* \* \*